

# UNITED STATES PATENT OFFICE.

OTTO P. AMEND, OF NEW YORK, N. Y.

## PROCESS OF DYEING ANILIN BLACK.

SPECIFICATION forming part of Letters Patent No. 499,410, dated June 13, 1893.

Application filed November 18, 1892. Serial No. 452,439. (No specimens.)

*To all whom it may concern:*

Be it known that I, OTTO P. AMEND, a citizen of the United States, and a resident of the city of New York, State of New York, have 5 invented a certain new and useful Process of Producing a Fast-Black Color on Fibrous Substances, of which the following is a specification.

Heretofore processes of printing or dyeing 10 in black upon vegetable fibers, as cotton, linen and mixed fibers, with aniline, toluidine and other aromatic amines and their salts, have produced fairly satisfactory results, but all attempts to produce a fast black with such 15 amines and salts upon animal fibers, especially wool and silk, have proved unsuccessful. Various processes have been tried, but none has produced a fast black. These failures have been attributed by some to a peculiar reducing action of the fibers during the 20 dyeing or developing of the black, and as the processes have depended upon oxidation of the dyeing material to produce the color this contemplated oxidizing effect has been counteracted by the reducing action of the animal 25 fibers. Others attribute these failures to the peculiar action of the fibers due to the sulphur contained in them, and various processes have been devised for a partial or complete elimination of this sulphur, but all such processes 30 have so far proved unsuccessful.

I have found that an aqueous solution of chromic acid in presence of another acid that will not produce a secondary oxidizing re-action 35 on the fiber, preferably hydrochloric or acetic acid, produces upon animal fibers a peculiar and very intimate union and combination, whereby the fiber is partially oxidized and part of the chromic acid is taken up by 40 it and apparently combines with it, forming a chromic compound with the fibers. It is necessary that the quantity of chromic acid in the solution be such that after a part is reduced to chromic oxide, a sufficient amount 45 remains to combine with the fiber. The presence of the second acid is necessary to keep in solution all of the chromic oxide formed and thus prevent its being deposited on the fiber. The acids which cannot be used in the 50 solution with the chromic acid are such acids

as sulphuric and nitric, which would oxidize or destroy the fiber.

The treatment of the animal fiber with the above mentioned solution of chromic acid in presence of other acids is the first step or re-action in my process of producing a fast black color. The second step or re-action of the process consists in treating the fiber with any of the aromatic amines or their salts in presence of a salt of metallic oxide, whereby a 55 fast black color is developed first in the cold and the development is finally completed at a heat of about 80° centigrade.

My new process is applicable to wool, silk and other animal fibers and also to vegetable 60 fibers, and may be applied to such fibers in any of their usual forms, as when in a separated state, or when twisted into yarns or threads or when woven into cloths or other fabrics.

I will now fully and particularly describe 65 my complete process.

I prepare an aqueous solution of chromic acid and hydrochloric acid and immerse the 70 wool or other fabric therein. The proportions 75 of acid for each one half kilogram of wool, are about twenty grams of anhydrous chromic acid and about thirty grams of hydrochloric acid. Sufficient water is employed to permit complete immersion of the fiber therein. The 80 solution is used at ordinary room temperature, from 20° to 30° centigrade. After the above described treatment the excess of the 85 solution is removed from the fiber by suitable mechanical means, such as wringing or pressing through rollers. The second solution is composed of aniline, toluidine or other aromatic amine or its salts which will produce 90 black and of metallic oxide salt, in the proportion for every one half kilogram of wool 95 or other fiber, of about fifty grams of the aromatic amine or salt and proportionate amount of the metallic oxide salt. Of the latter substances I have found that ferric sulphate produces very good results. Sufficient water is 100 employed to completely immerse the fiber. The solution is used at ordinary room temperature. After immersion in this second solution, the color begins to develop at the ordinary room temperature. After a certain

shade has been produced, the excess of the solution is mechanically removed, and the material is subjected to a temperature of about 80° centigrade. This may be accomplished 5 by placing the substance within a so-called Mather & Platt steam box or other heating device.

It will of course be understood that my invention is not limited to the exact proportions 10 above specified. For instance, the amounts of chromic acid and of hydrochloric acid above specified may be considerably exceeded without other result than a waste of such acids. So also some fibrous substances may require 15 slightly different proportions of the various aromatic amines, salts, and acids. Nor are the exact temperatures above described always essential to my invention. A beautiful deep black color is produced. The material as thus 20 colored will be found to withstand all the tests required of the best and most expensive blacks known. The fiber will be found to have lost none of its original physical properties, but on the contrary to have gained increased strength.

25 Having thus described my invention, what I claim as new, and desire to secure by Letters Patent, is—

1. The process of producing a fast black color on fibrous substances, which consists in 30 treating such substances with a solution of chromic acid in presence of other acid, that will not produce a secondary oxidizing effect

on the fibers and then treating such substances with a solution containing an aromatic amine or its salt, substantially as set forth. 35

2. The process of producing a fast black color on fibrous substances, which consists in treating such substances with a solution of chromic acid in presence of other acid, that will not produce a secondary oxidizing effect 40 on the fibers and then treating such substances with a solution of an aromatic amine or salt with a salt of metallic oxide, substantially as set forth.

3. The process of producing a fast black 45 color on fibrous substances, which consists in treating such substances with a solution of chromic acid in presence of another acid or acids, that will not produce a secondary oxidizing effect on the fibers then removing excess of said solution, then treating such substances with a solution of an aromatic amine or salt with a salt of metallic oxide, then permitting the black to partly develop at ordinary room temperature, then removing excess of said solution, then subjecting such substances to a higher temperature whereby such color is completely developed, substantially 50 as set forth.

OTTO P. AMEND.

Witnesses:

HENRY D. WILLIAMS,  
ROBT. A. KELLAND.